

Patented Oct. 2, 1928.

1,686,223

# UNITED STATES PATENT OFFICE.

PERCY A. E. ARMSTRONG, OF LOUDONVILLE, NEW YORK, ASSIGNOR TO LUDLUM STEEL COMPANY, OF WATERVLIET, NEW YORK, A CORPORATION OF NEW JERSEY.

## STABLE-SURFACE IRON-CHROMIUM-SILICON ALLOY.

No Drawing.

Application filed February 19, 1924. Serial No. 693,920.

My invention relates to a stable surface iron-chromium-silicon alloy, especially adapted to the production of rolled products, as for example, rolled bars, plates and sheets.

5 In the ferrous alloy of the present invention the carbon is kept as low as practicable and preferably under .05%, the presence of carbon being detrimental to the stable surface qualities and also to the workability of 10 the material.

The chromium of the alloy should be sufficiently high to give good working qualities.

A peculiar softening effect appears to set in 15 with the chromium-iron alloys with such low carbon, at about 13% of chromium. At about 16.5% chromium this softening effect seems to be as great as with still higher chromium. Higher chromium is, of course, 20 expensive and does not appear to add materially to the stable surface qualities.

Therefore, while I may use up to about 30% chromium, which is about as high a percentage as will be practically utilized, I prefer not to go over about 20% chromium.

25 I have found that within the broader range of about 13-30% chromium a narrower range of about 16-20% chromium can be used to great advantage and a still narrower range of about 16.5-18.5% chromium is preferable for securing desirable softness and 30 workability with the requisite stable surface qualities.

The silicon adds materially to the stable surface qualities, especially when the material is to be exposed to hot oxidizing gases, and also adds to the hot workability, the combination, essentially of iron, chromium and silicon, having the characteristics for 35 rolling, which are found in a pure metal made up of a single element. While the effects of silicon are to be noted with silicon as low as .30%, higher silicon of about .5-5% is preferably used. Silicon higher than about 2.5% is not desirable in large 40 cross-section bars or heavy rolled plate because of a tendency to resulting brittleness at atmospheric temperatures.

The principal part of the remainder is iron, though small percentages, preferably 45 not to exceed 5% each, of other metals may be present to give the properties normally resulting from such additions. For example, small additions of tungsten, molybdenum, manganese and nickel have a desirable toughening effect upon the alloy, where-

as larger additions of tungsten and manganese do not seem to convey any great benefit to the alloy. Nickel, however, in large percentages has a toughening effect but when used in excess of about 1%, difficulties are 60 encountered from the point of view of machinability; and manganese is particularly desirable up to about .50% as it adds slightly to the rollability at rolling mill temperatures; whereas higher manganese does not 65 seem to add anything to hot malleability of the alloy.

The preferred method of making this alloy is by heating substantially carbon free, or low carbon chromium or ferrochrome to a 70 fairly high heat (the higher the temperature the better, so long as it is below the melting point) and adding it to or adding to it, practically carbon free molten iron with suitable additions of substantially carbon free ferrosilicon or metallic silicon, which is also preferably highly heated, but not molten. It is essential in order to procure sound ingots or castings that the iron be degasified, preferably by aluminum, before the alloy addition is made. Instead of or adjunctive to making the silicon introduction separately, ferrochrome made by silicon reduction may be used containing suitable proportions of silicon. Where the heated chromium material is charged into molten iron the slag on the latter affords ample 75 slag for the former, but when the latter is added to the former, neutral slag may advantageously be thrown over the hot chromium material, or a slag heated up with the chromium material before making the iron addition. When adding manganese, tungsten, or nickel, or any other alloying material, same can be conveniently mixed with 80 the chromium and heated up therewith prior to adding it to or adding to it the molten substantially carbon free iron. This, however, is not a prime requisite because the percentage is relatively small.

85 The molten alloy is cast into ingot molds substantially as soon as it is completely melted, and the heat may be increased or maintained as by an addition of litharge or its equivalent in the furnace or ladle or mixer, the lead reduced sinking to the bottom and being usually found in the bottom of the first ingot cast. In this way carbon additions incident to time exposure of molten high chromium alloys to atmospheric 90 100 105 110

dust and to furnace, etc., linings, and the like are substantially completely avoided. Such process, which is applicable to the making of practically carbon free stable surface alloys with or without relatively high silicon is not claimed per se herein, being so claimed in my copending application Serial No. 675,306, filed Nov. 17, 1923, now Patent Number 1,557,132, dated October 13, 1925.

As an example, it has been found that material within the ranges referred to and showing upon analysis about 17% chromium, about 1% silicon and carbon about .03% is particularly well adapted for pack rolling into sheets. When pack rolling is resorted to, particularly for thin gauges, it is advisable to first give to the sheet a charcoal or similar wash, which gives a very good finish 20 on the pack side after rolling.

Stable surface alloy of analysis within my limits cannot be hardened to any substantial extent by heating and quenching. For example, an alloy containing chromium about 25 17%, silicon about 1%, carbon about .03%, manganese about .4% and the balance principally iron, when fully annealed has about 160 Brinell hardness, the same alloy as rolled or as air cooled is about 170 Brinell hard; 30 quenched from temperatures under 1900° F. about 170; and quenched from above about 1900° F. the Brinell hardness figure is about 220.

In commercial and quantity production, 35 the chromium-iron-silicon alloys within my limits are preferably hot finish rolled. During hot rolling, the material should be subjected to as much mechanical working as it is capable of withstanding. The toughness 40 of the material to impact is greatly increased in hot rolling by the use of heavy drafts at roll passes. It is undesirable when rolling from initial high rolling temperatures to use relatively light drafts at roll 45 passes, such as are generally used in rolling alloy steels such as high-grade tool steels, for example. With rolling mill equipment capable of producing the desirably great reduction at roll passes, the alloy may advantageously be heated up to fairly high initial 50 temperatures, for example, around 1900-2300° F. for the hot rolling. The finishing temperature for this rolling should be under about 1550° F., as with higher rolling 55 finishing temperatures, the tendency is to produce brittleness, which is apparently due to large grain size. This hot rolling with heavy passes may be advantageously finished at a temperature in the neighborhood of 60 1500-1400° F., or somewhat lower.

If desired, and especially if the mill equipment available for rolling the alloy is not capable of producing sufficient reduction between passes to obtain a good degree of 65 toughness in the manner just described, then

such high initial rolling heats should be avoided, or, in other words, the initial rolling temperature to which the alloy material is heated should be kept low. For example, with such relatively light draft rolling from relatively low initial temperatures the billets, blooms, sheet bars and the like for final rolling should be heated to a temperature in the neighborhood of 1500-1600° F., depending somewhat upon the amount of 70 total reduction to be given, and the finishing temperature should be under about 1400° F., and preferably under 1100-1200° F. The alloy has good hot malleability at about 1000° F., for example, and the rolling can 80 be carried down to atmospheric temperatures, if desired.

Quite different fractures are produced by the two described methods of working. The fracture of the alloy rolled at the high temperatures with the heavy reductions between 85 passes and the rolling finished at about 1450° F. or somewhat higher is substantially crystalline with a tendency toward lamination when a broken surface is visually observed 90 without the microscope. If in this hot rolling heavy work method the temperature of the finishing of the rolling step is carried low, say, for example, down to about 1300-1100° F. or lower, the structure becomes 95 more noticeably lamellar, this tendency being increased as the finishing temperature is lowered. The material in either case is quite tough, but still greater toughness to impact can be produced by reheating the bar, 100 plate, sheet or the like after finish rolling to a temperature where a new grain birth (not an accompaniment of passing through a critical temperature, but apparently a form of release of mechanical stresses) is 105 discernible, the laminations being practically obliterated, and the material is extremely tough. For example, in the case of such hot rolled products rolled at high temperatures using heavy drafts between passes, 110 with or without the low temperature finishing rolling, they may thus be reheated after finish rolling to about 1500-1600° F. and quenched in oil or water or allowed to cool 115 in the atmosphere or very slowly cooled, with resulting increase in toughness and in their notched bar impact value.

If, however, low initial temperatures and relatively light passes have been employed in finish rolling, the fracture is substantially 120 entirely lamellar in its nature, and it is undesirable to heat treat the alloy after rolling in such a way that this lamellar structure is substantially broken up, since, if this be done, it is brittle to impact and this is 125 apparently due to larger size crystal structure and intergranular weakness. The material when rolled at low temperatures and with relatively light passes is best reheated after rolling to about 1200-1300° F., and 130

quenched in oil, or water, cooled in the air or slowly cooled. With this treatment the laminations appear to be substantially preserved. Such treatment results in substantial removal of the strains from relatively cold working, and the rolled bar, plate or other rolled product is quite tough to notched bar impact testing. The modes of procedure above described are of especial advantage in finish rolling, but may be used to advantage from the ingot to the finished hot worked product. The alloy may be forged instead of rolled, and in forging the above stated relation of temperatures and vigor of working should be observed.

I claim:

1. The process of rolling stable surface alloys containing principally chromium, silicon and iron, with chromium over about 13%, silicon about .3-5%, with carbon as low as practicable and the principal part of the remainder iron, which comprises heating to a comparatively high rolling temperature and rolling same with substantially maximum draft roll passes.

2. The process of rolling stable surface alloys containing principally chromium, silicon and iron, with chromium over about 13%, silicon about .3-5%, with carbon as low as practicable and the principal part of the remainder iron, which comprises heating

to about 1900-2300° F., rolling with substantially maximum draft roll passes, and finishing the rolling at temperatures of about 1400-1500° F.

35

3. The process of rolling stable surface alloys containing principally chromium, silicon and iron, with chromium over about 13%, silicon about .3-5%, with carbon as low as practicable and the principal part of the remainder iron, which comprises heating to about 1900-2300° F., rolling with substantially maximum draft roll passes, finishing the rolling at temperatures of about 1400-1500° F., and reheating to about 1500-1600° F. and cooling.

4. The process of making wrought articles of alloys containing principally chromium, silicon and iron with chromium over about 13%, silicon about .3-5%, carbon as low as practicable and under .05%, which comprises putting together degasified molten iron and preheated chrome alloy material, casting into ingots, hot working into reduced sizes, heating to an initial rolling temperature of about 1900-2300° F., and finish rolling with substantially maximum draft roll passes, finishing the rolling at a temperature above about 1100° F.

50 55  
In testimony whereof, I have signed my name hereto.

PERCY A. E. ARMSTRONG.